

## UNITED STATES PATENT OFFICE

2,045,286

## METHOD OF STABILIZING REFLECTORS

Martin Tosterud, Arnold, Pa., assignor to Aluminum Company of America, Pittsburgh, Pa., a corporation of Pennsylvania

No Drawing. Application December 27, 1932,  
Serial No. 649,111

3 Claims. (Cl. 148—6)

The invention relates to reflecting surfaces of aluminum and to methods by which the reflecting power of such surfaces may be substantially stabilized.

The metal aluminum (or its aluminum-base alloys), when provided with a polished surface, is a very efficient reflector of radiant energy. For visible light, such a surface has a reflectivity of about 70 to 80 per cent, more or less. For infrared or heat radiation, the reflectivity of polished aluminum surfaces is about 90 per cent or more. The bright metal likewise has a very low emissivity. The metal is therefore used for reflecting surfaces and finds wide usage in lighting reflectors. Usually in the form of foil, aluminum finds application in insulating structures and is used as such in many places, including refrigerators, ships, trucks. In such usages the polished aluminum surfaces of low emissivity bound dead air spaces.

Reflecting aluminum surfaces are, in their wide and varied uses, placed in many environments. While under many conditions of service, the reflecting power of the aluminum surface is stable and remains constant, or substantially so, for long periods of time, there are other adverse service conditions where the reflectivity is unstable and tends to deteriorate gradually or even rapidly to values which are, comparatively speaking, very low. While the need for a treatment which would stabilize the reflectivity of polished aluminum surfaces has long been felt, such treatments as have heretofore been tried have been unsatisfactory for one reason or another.

The method of the present invention has been developed with the end in view of stabilizing the metal reflecting surface and it consists, in brief, of treating the bright aluminum surface in a hot solution of a class of salts herein termed chromates. The chromates are of two general types—the true chromates, which are the more efficient, and the dichromates. Both serve the purpose of the present invention, provided, of course, that they are appreciably soluble and do not attack the aluminum surface. The class of salts comprehended by the term "chromate" is, therefore, inclusive of the appreciably soluble chromates and dichromates. Of this class the alkali metal salts are preferable because of their ready availability, low cost, and high solubility, and such salts will be specifically referred to in the description of the methods of this invention.

The bright aluminum surface, the reflectivity of which is to be stabilized, is, in accordance

with the invention, treated with a hot solution of chromate. The exact physical method of bringing the solution to the metal surface is not important; suffice it to say that any method of application by means of which the bright aluminum surface is covered with the hot solution of chromate will be adequate. Dipping, spraying, brushing and the like are all possible processes, but in normal practice it is usually physically and economically convenient to simply immerse the metal in the hot solution. Another method which may prove convenient is that of spraying or otherwise placing a thin layer of chromate solution on the metal and then placing the wetted metal in a steam chamber or an oven where the high temperatures will quickly develop a high temperature at the interface between the metal and the chromate solution. The main variables to be considered are those of time of contact with the solution, concentration of chromate in the solution, and temperature of the solution. Of these variables, temperature is of major importance. The concentration of chromate in solution and the time of treatment are to some degree dependent, and generally a low concentration of chromate will require a longer time of treatment. But in any case, a comparatively short treatment, for instance one of 5 to 60 minutes, will suffice. The temperature of the solution is more critical. Hot solutions are preferably used, and when the article is immersed in such solutions the solutions are best held at approximately 75° centigrade or more. The boiling temperature is preferred since at this temperature the best results are obtained and likewise it is a solution temperature which is readily maintained constant.

The effects obtained in the treatment of bright aluminum surfaces by the methods of this invention are of a major order. The initial reflectivity of the aluminum surface is substantially maintained but the stabilizing effect of the treatment is such that decreases in reflectivity of the order of 50 per cent, as sometimes occur under severe conditions, are prevented for long periods of time.

As an example of the efficiency of the method of stabilizing the reflectivity of aluminum surfaces may be cited the following severe tests:

Aluminum sheet with a bright reflecting surface derived from being finished on polished rolls, was treated by the method of my invention. One lot was boiled for 30 minutes in a 10 per cent solution of potassium dichromate. The second lot was boiled for 15 minutes in a 10 per cent

solution of potassium chromate, and a third lot, without treatment, was included in the test. It is known that wetting of reflecting aluminum surfaces, or condensation under high humidity conditions is a severe test of the durability of reflecting surfaces, and for the present test, samples of the metal above-described were immersed in tap water for a period of one and one-half years, after which the samples were removed and their reflectivities measured. The original metal before treatment had a reflectivity of about 68 per cent. This reflectivity was not decreased by boiling in chromate solution. However, after one and one-half year's immersion in tap water, the untreated metal had its reflectivity decreased to 25 per cent, whereas the metal treated in dichromate solution had a reflectivity of 58 per cent, and the metal treated in chromate solution had a reflectivity of 63 per cent.

In another test, bright aluminum foil having a reflectivity of 80 per cent was treated for 10 minutes in a boiling 10 per cent solution of sodium chromate. The foil, after treatment, showed no loss in reflectivity. Samples of the treated and untreated foil were exposed in an atmosphere of 100 per cent humidity at about

30° centigrade, and under conditions which caused the surface of the foil to be continually wet with condensed moisture. After 100 hours' exposure under these conditions, the sample of untreated foil had turned quite dark and had a reflectivity of only 12 per cent, whereas the sample of foil treated with the sodium chromate solution had a reflectivity of 79 per cent, showing substantially no loss in reflectivity. 5

I claim:

1. The method of stabilizing the reflecting power of aluminum surfaces consisting of heating said surfaces in contact with a solution of a substantial amount of chromate in water. 10
2. The method of stabilizing the reflecting power of aluminum surfaces consisting of applying to said surface a solution of a substantial amount of chromate in water at a temperature of at least about 75° centigrade. 15
3. The method of stabilizing the reflecting power of aluminum surfaces consisting of applying to said surface a solution of a substantial amount of chromate in water at a temperature of at least about 75° centigrade for a period of 5 to 60 minutes. 20

25  
MARTIN TOSTERUD.